

1,338,779.

W. KLOCKE,  
METHOD OF FORGING,  
APPLICATION FILED MAY 16, 1919.

Patented May 4, 1920.

Fig. 1.



Fig. 2.



Fig. 3.



Fig. 4.



Fig. 5.



Fig. 6.



WITNESS :

*Rene' Prieur*

INVENTOR

*William Klocke,*

By Attorneys,  
*Draser, Durk & Myers*

# UNITED STATES PATENT OFFICE.

WILLIAM KLOCKE, OF NEW YORK, N. Y., ASSIGNOR TO PRESSED BEARING COMPANY, INC., OF BROOKLYN, NEW YORK, A CORPORATION OF NEW YORK.

## METHOD OF FORGING.

1,338,779.

Specification of Letters Patent. Patented May 4, 1920.

Application filed May 16, 1919. Serial No. 297,654.

To all whom it may concern:

Be it known that I, WILLIAM KLOCKE, a citizen of the United States of America, residing in Woodhaven, in the borough and 5 county of Queens, city and State of New York, have invented certain new and useful Improvements in Methods of Forging, of which the following is a specification.

This invention relates to the forging of 10 flanged structures or those consisting of a central portion in the nature of a hub surrounded by one or more outwardly turned flanges or webs. The method is peculiarly adapted to drop-forging.

15 In the accompanying drawings,—

Figure 1 is a side elevation of a billet;

Fig. 2 is a side elevation of the forging resulting from the first operation thereupon;

20 Fig. 3 is a mid-section of the forging dies and billet, illustrating the second operation;

Fig. 4 is a similar section illustrating the final operation for the formation of a forging having a single circular flange;

25 The remaining figures illustrate the application of the invention to the forging of objects having two such flanges.

Fig. 5 is a view of the billet resulting from the first operation, and corresponding to Fig. 2;

30 Fig. 6 is a section of the forging resulting from the second operation, corresponding to the forging shown in Fig. 3;

Fig. 7 is an elevation of the completed forging.

35 In practising the invention for the production of a single flanged hub or other similar forging, I proceed as follows:

A billet such as A (Fig. 1) is heated and placed between dies, and subjected to a blow 40 or pressure whereby it is upset to approximately the form shown at B in Fig. 2. This partly forged billet B is then placed in the cavity of a die C (Fig. 3) and is struck or pressed by a die D, whereby the 45 outer hub portion of Fig. 2 is indented by the annular conical portion d of the die D, and is squeezed out into the form of a conical flange c, the partly forged billet being here lettered E. This billet E is then 50 placed in a die F and is struck or pressed by a die G (shown in Fig. 4), whereby the conical flange c of Fig. 3 is forced out into a plane (in the example shown) perpendicular to the axis of the body portion of

the billet, as shown at h. The completed 55 forging is lettered H.

Heretofore, in the effort to produce such forgings as this forging H for use as the hubs of vehicle wheels and other purposes, it has been customary to form the flange h 60 solely by an upsetting process, the middle portion of the billet being squeezed outwardly in two, or perhaps three, upsetting operations. Difficulty has been found in 65 practice in thus making such forgings, because of the liability of the flanged middle portion of the forging, which is forced outward by the upsetting action, to crack or form fissures, or be otherwise defective, owing to the reluctance of the metal to flow and 70 yield to the squeezing-out tendency of the upsetting operation. This operation results in a violent increase of the exterior dimension of the flange, measured circumferentially, and any imperfection in the billet, 75 or any chilling below the most desirable temperature, is almost certain to result in radial cracks or other imperfections.

The improved method provided by the present invention results in a more gradual 80 operation and a less violent or forcible stretching of the marginal portion of the flange. By indenting in the manner shown in Fig. 3, the billet previously flanged out in the manner shown in Fig. 2, the flange 85 is reduced to so nearly its final dimension in thickness as to leave only about sufficient metal to form the finished flange, the outer portion of flange c being for this purpose made of greater thickness than its inner portion, and by this second operation it has been 90 carried out to nearly its final projection from the center, and hence to nearly its final circumferential dimension. The last squeezing operation, according to Fig. 4, is not in 95 the nature of an upsetting operation, but involves merely a further bending outward of the flange from conical form to flat or disk form. The middle of the flange is thus gradually shaped or "coaxed" outward. 100

To make a double-flanged hub or other similar forging according to the present invention, it is only necessary to duplicate the operations already described. This will be clear from Figs. 5, 6 and 7. In Fig. 5 the original ingot is shown in dotted lines at A', and the flanged ingot formed therefrom is shown in full lines at B', having two hubs

or enlargements  $b'$  and  $b''$  formed thereon. In Fig. 6 these have been pressed into conical flanges  $e'$  and  $e''$  in the same manner as the formation of the flange  $c$  in Fig. 3. The 5 incomplete forging of Fig. 6 is then placed within a divided die  $F'$ , shown in dotted lines in Fig. 7, and dies corresponding to the die  $G$  in Fig. 4 are brought against it from opposite sides, whereby the flanges  $e'$   $e''$  are pressed into the final disk form of the flanges  $h'$   $h''$  of Fig. 7, thereby forming the finished double-flanged forging  $H'$ .

The invention may be modified by making the successive steps more or less gradual, and 15 by varying the shape of the dies to accord with any desired shape of forging that it is intended to produce. In general, the method may be varied in any manner which will adapt it to the requirements of practice, as will be apparent to those skilled in 20 the forging art. In the references herein to the flanges  $e'$   $e''$  as "conical flanges," I am not to be understood as being limited to these flanges being of precisely conical form, since 25 any form approximating a cone is to be considered within the invention.

The indenting operation shown in Fig. 3, is performed solely by the die  $D$ , which acts within the flange  $c$ , there being no squeezing 30 out of the flange between two dies so that by flowing the metal fills the space between them, as has heretofore been done.

I claim as my invention:—

1. The improved method of forging which 35 consists in partly upsetting a billet to form a thickened portion thereon, then annularly indenting such thickened portion to form a conical flange, and finally flattening such conical flange.
2. The improved method of forging which 40 consists in forming a billet with a thickened end, then indenting said thickened end to squeeze its outer portion outwardly into con-

ical form, and finally subjecting said conical portion to pressure between dies to press it 45 further outwardly and to reduce its thickness to form an outwardly directed flange.

3. The improved method of forging which consists in forming a billet with a thickened end, then annularly indenting said billet 50 to squeeze its outer portion outwardly into conical form, while leaving its central portion of substantially its former length, and finally subjecting such conical portion to pressure to bring it to final form. 55

4. The improved method of forging which consists in forming a billet with a thickened portion, then annularly indenting such thickened portion to squeeze it outwardly into the form of a conical web by means of 60 an annular die having an external conical face engaging the inner side only of the outwardly displaced metal.

5. The improved method of forging which consists in indenting a billet near its exterior 65 by pressure from one end only to squeeze the outer portion of metal outwardly into the form of an approximately conical web, by means of a die engaging only the inner side 70 of the displaced metal.

6. The improved method of forging which consists in indenting the end of a billet by means of a die entering said end whereby to squeeze the metal outwardly into conical form, the outer portion of the displaced 75 metal being formed of greater thickness than its inner portion.

7. The improved method for producing a double-flanged forging which consists in annularly indenting opposite end portions of 80 a billet to form two conical flanges thereon, and subsequently flattening such conical flanges.

In witness whereof, I have hereunto signed my name.

WILLIAM KLOCKE.